

## UNITED STATES PATENT OFFICE

ROBERT JAY SHOEMAKER, OF CHICAGO, ILLINOIS, ASSIGNOR TO S. & T. METAL COMPANY, OF CHICAGO, ILLINOIS, A CORPORATION OF ILLINOIS

## LEAD ALLOY

No Drawing. Application filed November 28, 1928. Serial No. 322,573.

This invention relates to lead alloys and its primary object is to provide an alloy of lead having certain characteristics that make it particularly suitable for the manufacture of pipes, cable coverings, battery plates, linings for acid tanks, and for other like purposes. These characteristics comprise a degree of hardness greater than that of pure lead but not enough to prevent working the metal by cold processes; and very considerable increase in tensile strength in comparison with lead; and a higher resistance to the corrosive or solvent effect of acids.

Another object of the invention is to provide a lead alloy, of the general character above indicated, from which the alloying metals will not drop out in case it is necessary to melt the alloy and which will be substantially non-corrosive in moist atmospheres.

The compound consists principally of lead. The alloying metals are used only in very small quantities. The substance which may be termed the primary hardener is calcium. A small quantity of aluminum is used, preferably, to prevent the dropping of the calcium in the making of the compound, and later in case it is necessary to melt the alloy. However, it would be possible though inconvenient to protect the batch against oxidation during compounding and if the alloy were to be fabricated subsequently by processes not involving melting and in this case the aluminum would not be an essential element. In addition to the primary hardener, calcium, the alloy contains one or more substances that may be termed secondary hardeners because they produce a greater increase of hardness when incorporated in a lead-calcium alloy than when they are used alone with lead. These secondary hardeners comprise tin and mercury, used either singly or together.

The following table indicates preferable

limits in respect to the proportions of the ingredients:

|                       | Per cent    |
|-----------------------|-------------|
| Calcium               | 0.1 to 0.4  |
| Tin                   | 0.5 to 2.0  |
| Mercury               | 0.1 to 1.0  |
| Aluminum              | 0.02 to 0.1 |
| Lead to make up 100%. |             |

The following is a specific and preferred example of the type of alloy contemplated by the invention:

|                       | Per cent |
|-----------------------|----------|
| Calcium               | 0.2      |
| Tin                   | 1.0      |
| Mercury               | 0.1      |
| Aluminum              | 0.05     |
| Lead to make up 100%. |          |

A pipe if made of this alloy will withstand bursting pressures substantially double those which ordinary lead pipes of corresponding weight will withstand. For example, a one inch lead pipe of four pounds to the linear foot should withstand bursting pressures up to 900 pounds per square inch. A pipe of the same diameter, but of two pounds per linear foot, if composed of the alloy described, will withstand pressures up to 900 pounds per square inch.

A pipe made of this alloy is cheaper, heavier, more durable and more flexible than a copper or brass pipe of the same diameter. The alloy has a hardness of approximately 5 Brinell, about twice the hardness of lead. The hardness may be varied by increasing or decreasing the primary and secondary hardening agents within the limits above indicated. Like degrees of hardness may be obtained by decreasing the calcium content and increasing the amount of tin or mercury or both.

It may be said that the tin may be used in considerably larger quantities than indicated in the table, but any substantial ex-

cess over 2% has no hardening effect, and on the contrary, seems to make the alloy somewhat softer. Tin being much more expensive than lead, the use of larger amounts of tin than indicated involves a useless economic waste. However, in fixing the upper limit of the tin at 2%, I do not wish to be understood as precluding the use of a larger quantity, although, for the reasons stated, there would be no advantage but on the contrary a disadvantage in such procedure.

The alloy is preferably made as follows: The lead is melted and heated to a temperature of approximately 1500° Fahrenheit under a covering of calcium chloride or other suitable flux. Aluminum is introduced, preferably as a 50% alloy of aluminum and tin. Since the amount of the aluminum is very small, the tin introduced in this way is practically negligible. The calcium, as metallic calcium, is then introduced into the lead. The melt is allowed to cool to a temperature just above the melting point of lead, say to 700° Fahrenheit, and the calcium chloride covering is skimmed off. Or the bath can be allowed to solidify and then remelted to about 700° Fahrenheit, whereupon in either case the mercury and tin are added.

The aluminum is used as an anti-drossing agent to prevent oxidation of the calcium. Its use in amounts in excess of the upper limit specified above has no advantage and tends to make the alloy porous and bring out excessive shrinkage losses.

When the alloy is used for making pipe, the pipe can be formed by extrusion, although higher pressures are required than are commonly used in making lead pipe.

If desired, the alloy may be compounded in part by an electrolytic process. The lead is melted and aluminum added. The melt is covered with calcium chloride and subjected to an electric current, the positive electrode being immersed in the calcium chloride and the negative electrode in the lead. The calcium chloride is split up, the calcium going into the lead and the chlorine escaping. The other ingredients are then mixed into the batch, after the latter is cooled to approximately 700° Fahrenheit as in the other process.

The alloy as specified under Example 1 may be modified as follows:

#### Example 2

The mercury given under Example 1 is omitted and the calcium content increased. A preferred formula (subject to modification within the limits given in the first table above) is as follows:

|                       | Per cent |
|-----------------------|----------|
| Calcium               | 0.3      |
| Tin                   | 1.0      |
| Aluminum              | 0.05     |
| Lead to make up 100%. |          |

While specific examples have been given, it is intended to cover by patent all modifications within the scope of the appended claims. In using the term "consisting essentially" in the claims I do not intend to exclude the possibility of incorporating in the alloy other substances of such a character or in such small amounts as not to substantially affect the character of the alloy as described above.

I claim:

1. A tough, slightly hardened, non-corrosive lead alloy consisting principally of lead and containing the following substances in quantities by weight substantially as follows: calcium 0.1 per cent to 0.4 per cent and tin 0.5 per cent to 2.0 per cent.

2. A tough, slightly hardened, non-corrosive lead alloy consisting principally of lead and containing the following substances in quantities by weight substantially as follows: calcium 0.1 per cent to 0.4 per cent and tin 0.5 per cent to 2.0 per cent and mercury from 0.1 per cent to 1.0 per cent.

3. A tough, slightly hardened, non-corrosive lead alloy consisting principally of lead and containing the following substances in quantities by weight substantially as follows: calcium 0.2 per cent and tin 1.0 per cent.

4. A tough, slightly hardened, non-corrosive lead alloy consisting principally of lead and containing the following substances in quantities by weight substantially as follows: calcium 0.2 per cent, tin 1.0 per cent and mercury 0.1 per cent.

5. A tough, slightly hardened, non-corrosive lead alloy consisting principally of lead and containing the following substances in quantities by weight substantially as follows: calcium 0.1 per cent to 0.4 per cent, tin 0.5 per cent to 2.0 per cent and aluminum from 0.02 per cent to 0.1 per cent.

6. A tough, slightly hardened, non-corrosive lead alloy consisting principally of lead and containing the following substances in quantities by weight substantially as follows: calcium 0.1 per cent to 0.4 per cent, tin 0.5 per cent to 2.0 per cent, mercury from 0.1 per cent to 1.0 per cent, and aluminum from 0.02 per cent to 0.1 per cent.

7. A tough, slightly hardened, non-corrosive lead alloy consisting principally of lead and containing the following substances in quantities by weight substantially as follows: calcium 0.2 per cent, tin 1.0 per cent and aluminum from 0.02 per cent to 0.1 per cent.

8. A tough, slightly hardened, non-corrosive lead alloy consisting principally of lead and containing the following substances in quantities by weight substantially as follows: calcium 0.2 per cent, tin 1.0 per cent, mercury 0.1 per cent, and aluminum from 0.02 per cent to 0.1 per cent.

9. A tough, slightly hardened, non-corrosive lead alloy consisting principally of lead

and containing the following substances in quantities by weight substantially as follows: calcium 0.2 per cent, tin 1.0 per cent and aluminum 0.05 per cent.

10. A tough, slightly hardened, non-corro-  
5 sible lead alloy consisting principally of lead and containing the following substances in quantities by weight substantially as follows: calcium 0.2 per cent, tin 1.0 per cent, mercury 0.1 per cent, and aluminum 0.05 per cent.

10 ROBERT JAY SHOEMAKER.

15

20

25

30

35

40

45

50

55

60